

## UNITED STATES PATENT OFFICE

2,129,844

METHOD OF MAKING BEARING AND GAS-  
KET MATERIALEdwin F. Kiefer, Cleveland, Ohio, assignor, by  
mesne assignments, to Union Carbide and Car-  
bon Corporation, a corporation of New YorkNo Drawing. Application July 21, 1934,  
Serial No. 736,344

7 Claims. (Cl. 75—22)

This invention relates to a method of making porous structures and especially impregnated porous structures suitable for use as gaskets, bearings, or the like.

5 An object of this invention is to provide a hard, porous base or matrix which is capable of being impregnated with softer materials. Another object of this invention is to provide a method of producing a base or matrix having a large number of fine pores. Still another object is to provide a bearing or gasket of porous copper impregnated with softer materials. The above and other objects together with the novel features of this invention will be apparent from the following description.

To achieve the above-enumerated objects in accordance with this invention, a matrix is first prepared from a suitable metal or its oxide. Any oxide of a metal may be used which is capable 20 of being reduced and at the same time of being formed into a coherent mass in the manner of a porous honeycombed structure. However, it is preferred to employ copper and/or copper oxide in forming a matrix because of inherent characteristics peculiar to this metal. Desirable results are obtained with a comminuted mixture 25 of copper and copper oxide, but copper or copper oxide alone is also suitable. The copper and copper oxide may be finely divided or pulverized and 30 intimately mixed with a suitable reducing agent. Ammonium chloride provides the necessary chemical constituents to perform the reducing reaction and also acts as a binder to cause the copper and copper oxide particles to adhere closely 35 together. The limiting proportions of  $\text{NH}_4\text{Cl}$  are 0 to 18% but I prefer to use from 4 to 15%. Above 18% there is a decided tendency for the 40 formed article to crack and deform. Below 4% the reduction is insufficient to produce a well bonded uniform structure.

The mixture of copper, copper oxide, and ammonium chloride is molded in a form and compressed into sheets or other convenient shapes. When the sheets are so prepared they are next 45 placed in an oven, muffle, or other heat-producing equipment and sintered. The temperature of the oven is raised to substantially 900° C., at which temperature it is found that the reducing reaction will occur most speedily and efficiently. An inert atmosphere, from which oxygen has been excluded, materially aids in making the reaction complete, and it has also been found that an increase in pressure above atmospheric will tend to assist in speeding the baking process. 55 The baking acts to sinter the molded sheets of

powdered copper, leaving a porous, closely knit copper matrix.

During the heating, the ammonium chloride reacts with the copper oxide reducing the latter. The reaction is believed to be as follows:



Considerable ammonium chloride is volatilized and does not enter the reaction. However, the volatilized ammonium chloride serves as a blowing agent to produce porosity as well as to prevent oxidation. This results in the sheets or molded material becoming honeycombed or filled with pores. The copper particles become fused together at intermediate points throughout the mass and form a substantially rigid foraminous matrix which is not subject to crumbling nor to crushing under moderate pressure.

When the sheets have cooled, they are suitable for use as gaskets in their then existing form. However, superior gaskets may be made by impregnating the porous matrices with gums, resins, or waxes, or with softer metals such as 20 tin or lead.

I have found that lead and lead-tin alloys are 25 well adapted for this impregnation. This is best applied by soaking the porous matrix in molten lead or lead-tin alloy. The amount of lead taken up may vary from 6% for copper having a low porosity to as high as 105% for copper having a 30 higher porosity. When resins or the like are used as impregnating material, the percentage will be much lower. Other suitable materials may be used for impregnation, such as rubber, vinyl polymers, phenol formaldehyde condensation products, and the like. In nearly all instances I prefer to use the largest amount of impregnating material that the foraminous matrix will take up; that is, the foraminous matrix is 35 preferably substantially saturated with the impregnating material. In most cases immersion in the molten material is sufficient. However, if the introduction of more material is required, or if the material is viscous and does not penetrate with ordinary soaking, pressure methods can be 40 resorted to.

A matrix of copper which has been prepared in accordance with this invention and impregnated with lead or tin or alloys of soft metals is admirably suited to serve as a bearing material. 50 The relatively hard structure of the matrix withstands the high pressures which are experienced in the contact of metal parts movable in relation to other and cooperating parts. The softer impregnated material serves as an antifriction 55

medium and as a partial binder so that a hard, long-wearing and shock-resistant bearing is assured as well as one that will not crack or fail under severe compressive stress.

5 When the matrix is impregnated with gums, resins, graphite, or wax, it makes a suitable gasket or packing material. The softer filler substance tends to flow to the surface of the sheet and prevents leaks from occurring in glands, 10 stuffing boxes, and between metal edges, as in engine blocks and tank covers.

Although a preferred method and resulting gasket and bearing materials have been described, it will be understood that changes may 15 be made without departing from the principles or scope of this invention.

I claim:

1. A method of making a porous structure comprising the steps of mixing an unalloyed finely 20 divided oxide of copper with an ammoniacal salt; molding the mixture to a desired shape; and sintering the molded ingredients to form a porous mass of substantially pure copper.

2. A method of making a porous structure comprising the steps of mixing comminuted copper and copper oxide with ammonium chloride; molding the mixture to a desired shape; and heating the molded ingredients to create a coherent porous material.

30 3. A method of making an impregnated bearing comprising the steps of mixing an unalloyed pulverulent oxide of copper with ammonium chloride; molding the mixture; heating the molded ingredients to form a porous structure of

substantially pure copper; and introducing a softer metal into the pores.

4. A method of making an impregnated gasket comprising the steps of mixing unalloyed pulverulent copper with ammonium chloride; molding 5 the mixture; heating the molded ingredients to form a porous structure of substantially pure copper; and introducing an alloy of lead and tin into the pores.

5. A method of making an impregnated material 10 suitable for use as gaskets, bearings or the like, comprising the step of mixing comminuted copper and copper oxide with 4 to 18% ammonium chloride; molding the mixture; heating the molded ingredients in a reducing atmosphere 15 to form a foraminous structure; and introducing a softer substance into the pores.

6. A method of making an impregnated material comprising the steps of mixing an unalloyed pulverulent oxide of copper with a combined 20 blowing and reducing agent; molding the mixture; heating the molded ingredients in a reducing atmosphere to produce a sintered structure of substantially pure copper; and introducing from 6 to 105% by weight of an alloy predominantly 25 lead into the pores.

7. A method of making an impregnated material comprising the steps of mixing a pulverulent oxide of copper with ammonium chloride; molding the mixture; heating the molded article in a 30 reducing atmosphere to form a porous structure; and introducing a lead-tin alloy into the pores.

EDWIN F. KIEFER.